

Sept. 3, 1940.

J. W. ERB

2,213,759

METHOD OF MAKING SHEET METAL

Filed March 9, 1938

Fig. 1.



Fig. 2.



Fig. 3.



Fig. 4.



Fig. 5.



Fig. 7.



Fig. 6.



Fig. 8.



INVENTOR

John W. Erb

by his attorneys

Stebbins, Blenko & Parmele

## UNITED STATES PATENT OFFICE

2,213,759

## METHOD OF MAKING SHEET METAL

John W. Erb, Martins Ferry, Ohio, assignor to  
 Wheeling Steel Corporation, a corporation of  
 Delaware

Application March 9, 1938, Serial No. 194,876

1 Claim. (Cl. 148—4)

This invention pertains to the manufacture of sheet metal and, in particular, to so-called "blued" sheet steel having a tightly adherent skin of oxide extending uniformly over the surface thereof.

Blued sheet steel has customarily been made by admitting an oxidizing agent such as steam to steel sheets or strip while the latter are at an elevated temperature. It is usually preferable to 10 perform the oxidation step as one of the later stages of the usual annealing process. In such process, the sheet metal is usually disposed in the form of stacks of sheets or relatively tight coils of strip. Because of the manner in which 15 the sheet material is disposed for annealing it is not always possible to obtain uniform oxidation thereof because the oxidizing agent does not have easy access to the inner portions of the surface of sheets in stacks or strip in coils. As 20 uniformity in appearance of a product is an essential for most uses of blued stock, this problem is a very serious one.

I have invented a method of making blued stock whereby the aforementioned objection to the 25 previous practice is eliminated. In a preferred practice of the invention I provide for easy and uniform access of the oxidizing agent to all portions of sheets in stacks or strips in coils by so roughening the surface of the material prior to 30 annealing that even when successive layers of stacked or coiled material engage each other with considerable pressure, there is sufficient space therebetween to permit infiltration of an oxidizing agent such as steam. A preferred practice of the invention will be described in detail 35 herebelow with reference to the accompanying drawing illustrating the several steps diagrammatically. In the drawing:

Fig. 1 illustrates the step of rolling pickled hot 40 rolled strip to the desired finished gauge;

Fig. 2 represents the scrubbing treatment to which the material is then subjected;

Fig. 3 illustrates the initial annealing operation;

Fig. 4 illustrates the step of roughening the 45 surface of the material by rolling;

Fig. 5 is a plan view with parts omitted showing the result produced by this operation;

Fig. 6 illustrates the second annealing operation during the cooling stage of which the oxidizing agent is admitted;

Fig. 7 is a partial sectional view through a coil showing the relative positions of successive wraps thereof; and

Fig. 8 illustrates the final operation which re-

stores a smooth surface and bright finish to the material and gives it the temper which is desirable for subsequent fabricating operations.

Referring now in detail to the drawing, I preferably take a coil of pickled hot rolled strip 10 5 such as low carbon steel strip and subject it to cold reduction to the desired final gauge. This reduction may be effected by passing the material through tandem rolling mills 11 which are illustrated as of the 4-high type. It will be understood, however, that the strip may be reduced to gauge by any other suitable form of mill which may be available. The reduction effected by the mills 11 is usually greater than 50%. Typical starting and finishing gauges are 14 15 gauge and 30 gauge respectively. These gauges are cited simply by way of illustration as the invention may be applied to material varying in thickness.

After the strip has been rolled to the desired 20 final gauge, it is passed through a scrubber 12 as shown in Fig. 2 for the purpose of cleaning the surfaces thereof. The material is then in condition for annealing. This operation may be carried out in a furnace such as that shown at 13 in 25 Fig. 3 or any other suitable form of annealing furnace. In the initial annealing operation, the material is preferably heated to a temperature of between 1200° and 1300° F. A de-oxidizing atmosphere is preferably maintained, by means 30 already wellknown, in the annealing box 14 in which the material is enclosed as shown at 13, during the cooling stage of the operation.

After the initial annealing operation, I subject the strip to a so-called "dulling" pass as 35 illustrated in Figures 4 and 5. In this operation, the material is passed through a mill 16 which may also conveniently be of the 4-high type, the working rolls whereof have their surfaces roughened as by sand blasting or the like. The effect 40 of passing the material between the roughened work rolls of the mill 16 is to impart a considerable degree of roughness to the surface of the material, as indicated in Fig. 5. Little or no reduction in the thickness of a material is effected 45 by the mill 16.

After the surface of the material has been roughened suitably by passing it through the mill 16 or otherwise, the strip is coiled and again annealed, as illustrated in Fig. 6 in a furnace 17 50 similar to that shown at 13. During this annealing operation, the coils indicated at 18 disposed in an annealing box 19 are heated to a temperature of between 1000° and 1100° F., and after a suitable soaking period, are withdrawn 55

from the furnace for slow cooling. When the coils have cooled slightly below the maximum temperature attained during the second annealing, an oxidizing agent such as steam is admitted 5 to the box 19 by means already wellknown. The steam has access to all portions of both surfaces of the strip, even though the coils are tightly wrapped, because the roughness imparted to the strip surfaces leaves spaces between adjacent 10 wraps sufficient to permit the infiltration of steam therebetween. This condition is illustrated, somewhat exaggerated, in Fig. 7 wherein the successive wraps of a coil are indicated at 20. By reason of the roughness imparted to the 15 surfaces of the strip, adjacent wraps have close contact at spaced points only, leaving sufficient clearance for the entry of an oxidizing agent such as steam. An atmosphere of the oxidizing agent is maintained about the coils for a period 20 sufficient to effect the formation of a uniform coating of tightly adherent blue oxide. The resulting oxidation is substantially uniform throughout the surface of the strip because the oxidizing agent has ready access to all portions 25 as a result of the spaces between adjacent wraps provided by roughening the strip surfaces before the final annealing and oxidizing treatment.

When the oxidizing treatment has been completed, the coils are subjected to a final temper 30 pass in a rolling mill 21 having work rolls with smooth, highly polished surfaces such as that characterizing the work rolls 11. This temper pass rolls out the roughness imparted to the strip by the mill 16 and the resulting product is characterized by a smooth surface and a bright, lustrous finish. The temper pass also serves to increase the stiffness of the material sufficiently to prevent fluting when formed into cylinders.

It will be apparent from the foregoing description 40 that the method of my invention is characterized by an important advantage over the processes employed heretofore in the manufacture

of blued stock in that the oxidizing agent has relatively free access to all parts of the strip surface whereby the degree of oxidation and coloration is substantially uniform throughout the surface of the strip. The resulting increase in uniformity of the final product provides a greater percentage of prime material. The operations involved in the method of my invention are simple and may be carried out at relatively low cost with 10 existing equipment.

As a possible alternative to the specific practice disclosed herein, I contemplate using roughened work rolls in the last mill 11 so that a special "dulling" pass and a second annealing illustrated in Figures 4 through 6 may be eliminated.

Although I have illustrated and described but a preferred practice of the invention, changes and modifications therein may be made without departing from the spirit of the invention or the scope of the appended claim.

I claim:

In a method of making blued sheet steel, the steps including rolling the steel substantially to the desired final gauge, passing the sheet steel between roughened rolls, thereby imparting roughness to the material to such an extent as to permit access of an oxidizing agent to substantially all portions of the surfaces of the material when it is disposed in multiple thickness, heating the material in multiple thickness to a temperature at which it oxidizes rapidly in the presence of an oxidizing agent, admitting such agent in the neighborhood of the heated material while at said temperature, thereby forming a tightly adherent coating of oxide on the material and substantially uniformly bluing all portions thereof, by the infiltration of said agent between adjacent thicknesses of metal, and finally rolling the blued steel to produce a smooth surface without breaking said oxide coating.

JOHN W. ERB.